

# UNITED STATES PATENT OFFICE.

EDGAR M. BERLINER, OF MONTREAL, QUEBEC, CANADA.

## PROCESS OF MAKING SOUND-RECORDS.

1,355,791.

Specification of Letters Patent.

Patented Oct. 12, 1920.

No Drawing.

Application filed December 17, 1919. Serial No. 345,575.

To all whom it may concern:

Be it known that I, EDGAR M. BERLINER, a citizen of the United States of America, and a resident of Montreal, in the Province 5 of Quebec, Dominion of Canada, have invented certain new and useful Improvements in Processes of Making Sound-Records, of which the following is a specification.

10 This invention has reference to the production of sound-records and relates more particularly to the manufacture of that type of sound-records in which the phonetic characters of a matrix are reproduced in intaglio in a substance or composition which in the art is designated as the surface coating or glaze of the record.

Heretofore, sound-record tablets have been produced by the application of a glaze 20 or surface coating to the matrix, and also to the surface of the base of the tablet or disk, the different layers of material being united by heat and pressure, and in some instances a powdered glaze which consists 25 principally of shellac has been applied to the surface of the matrix by means of a sieve. Another known method having for its object the production of sound-records, involves the use of a mixture that is rolled 30 upon the negative matrix. The foregoing methods or processes are typical of those known or in use and disclose various attempts that have been made to obviate or avoid the presence of air bubbles or pits in 35 the commercial records, as well as efforts to produce perfect reproductions of the matrix, without the employment of methods and materials the cost of which would be prohibitive.

40 The object of my invention is to provide the matrix with a coating, particularly that part of the matrix which contains the phonetic characters, which coating will be free from pits, air bubbles, cavities and the like 45 and which coating is a perfect intaglio reproduction of the phonetic characters of the matrix. The result is accomplished by eliminating moisture, air, gas or any particles from between the matrix and the surface 50 that is being formed, also eliminating air or gas from the coating material itself. This intaglio provides a sound-groove in the commercial record in which such defects in reproduction as result from foreign loose particles as dust, and from the trapping of air

or gas between the matrix and the coating are eliminated.

My method or process not only eliminates in the product or sound-record, imperfections which are incident to a perfect reproduction of the phonetic characters of the matrix, but has other advantages among which may be mentioned, the use of less coating material, a gain in the rapidity of production, less wear of the matrix, and a 65 more perfect record surface.

My method or process consists in projecting record surfacing material against the matrix with force sufficient to dislodge air, gases, and foreign particles from the matrix, 70 to form a unified coating upon the matrix to which it adheres and from which it may not of itself be readily separated and handled. It subsequently becomes a part of a sound record tablet. When this coating or 75 film is applied to the matrix it provides a protective covering and eliminates to a great extent wear of the matrix incident to the movement of a plastic under pressure against the matrix. The coating may be 80 reinforced for handling by projecting other material thereon while still in contact with the matrix, but it is preferably united by heat and pressure with a base that is applied while the film-like coating is still in contact 85 with the matrix, separation from the matrix taking place on cooling. The application of the coating or surfacing material against the matrix involves the use of air, fluid or liquid under pressure or compression, to project the coating or surfacing material 90 against the matrix.

The preferred material that I use, is shellac which may be dissolved in alcohol, though I may use as a coating material for 95 the matrix, any suitable material in a fluid or solution state or form which may be projected with force against the matrix and when so projected adheres thereto, successive or further impacts will tend to force the material into intimate adherence with the matrix to give the desired result. I do not limit myself to the application of a liquid or fluid material as a coating or surfacing material for the matrix, as shellac 100 in a dry and pulverent or powdered form, with or without other substances may be successfully applied when projected with sufficient force upon or against a heated matrix to form a unified coating. The force 110

used is such as to give a high velocity to the material. Any of the coating material which may rebound from the matrix, or any other surplus, may be collected for reuse, 5 it also being within the scope of my invention to recover such solvents as may be employed to liquefy the shellac or other coating material. In practice, the coating material that is to be projected and impacted is 10 preferably first reduced to a liquid state, in which it may be heated; under pressure it is then sprayed, jetted or projected against the matrix, the material moving with high velocity strikes the matrix with considerable 15 force, and produces a perfect intaglio of the matrix.

The surface coating material, is sprayed, jetted or projected against the matrix, either from a single orifice, or from a plurality of 20 orifices. When the matrix or the source that emits the coating material is movable, or when the pressure that is applied to the coating material is varied, a stream or spray may result.

25 The surfacing material may be applied in a heated condition to the matrix. It may be applied to a heated matrix. Successive coats of the same material or of different materials may be applied in the manner 30 herein set forth.

In practice the coating material may be directed against the matrix so that the direction of impact will be in line with the phonetic characters thereon, or the raised 35 portion of the matrix which forms in the record the sound groove, or spirally with reference to the center, or perimeter of a disk tablet.

I claim:

40 1. The process of producing sound-records from a matrix having phonetic characters thereon which consists in forcibly projecting a record surfacing material against the matrix and uniting same with a base 45 while still in contact with the matrix.

2. A step in the process of producing sound-records from a matrix having phonetic characters thereon which consists in jetting a record surfacing material 50 against the matrix.

3. The process of producing a sound-record surface by forcibly projecting record surfacing material against a matrix having phonetic characters thereon, to form an intaglio thereof which is united with a base by 55 heat and pressure while still in intimate adherence with the matrix.

4. The process of producing a coating of record surfacing material on a matrix having phonetic characters thereon which consists in forcibly projecting a surfacing material against the matrix and subsequently applying such coating, while on the matrix, to a base by heat and pressure, separation 60 from the matrix taking place on cooling.

5. The process of forming sound-records from a matrix which consists as a step in the process in projecting record material in the form of a stream against the matrix.

6. The process of forming sound-records 70 from a matrix which consists in projecting a layer of surfacing material against the matrix, and then projecting one or more layers of other material thereon.

7. The process of forming a sound-record 75 tablet from a matrix which consists as a step in the process in coating a sound-record matrix with a coating the outer surface of which is substantially parallel to the irregular surface of the matrix. 80

8. The process of forming a sound-record from a matrix which consists as a step in the process in applying to a matrix a film-like coating the thickness of which is less than the greatest depth of the negative 85 sound groove.

9. The process of forming a sound-record surface from a matrix having phonetic characters thereon which consists in forcibly projecting record material in fluid condition 90 against the matrix and uniting the same with a plastic base while still attached to the matrix.

10. The process of forming a sound record 95 surface by successive impacts of record material against a sound record matrix and against each other, uniting the same with a base by heat and pressure, while still in contact with the matrix, and separating the sound record so formed, from the matrix, by 100 cooling and relieving the pressure.

11. The process of forming sound-records from a matrix which consists in spraying record surfacing material against the matrix. 105

12. The process of forming sound-records from a matrix which consists as a primary step in the process in impacting a record surface in the form of spray against the negative sound record matrix. 110

13. The process of forming sound-records from a matrix which consists in spraying a heated surfacing material against the matrix.

14. The herein described process of coating 115 a matrix with a sound-record surfacing material which consists in projecting in the form of spray a heated resinous material the force of the impact of the material against the matrix being such as to reproduce the sound-record thereof in said resinous material.

15. The herein described process of forming the record surface of a sound record from a matrix which consists in spraying a 125 comminuted resinous material with sufficient force to coat the matrix and to expel from the material by successive impacts, air bubbles, pits, and the like, to produce in the solidified coating or glazing a reproduction 130

- of the matrix and more particularly of the raised portion of the matrix which carries the phonetic characters, and in associating such sound-record with a backing.
- 5 16. The process of forming sound-records from a matrix which consists in impacting against the matrix a comminuted record surfacing material.
- 10 17. The process of forming sound-records from a matrix, which consists as a step in the process in impacting a record surfacing material in comminuted form against the sound-record face of the matrix.
- 15 18. The process of forming sound-records from a matrix, which consists as a step in the production of the sound-record in impacting a comminuted surfacing material against the sound-record matrix and then transferring under heat and pressure the
- 20 surfacing material to a sound-record base.
19. The process of coating a sound-record matrix with a surfacing material which consists in projecting and impacting a resinous surfacing material against the matrix to 60
- 25 produce the sound-record of the matrix and then associating the surfacing material on the matrix with a sound-record base.
20. The process of coating the face of a sound-record matrix which consists in spraying 70
- 30 a heated resinous surfacing material against the matrix and then associating the surfacing and record carrying material with a backing.
21. The process of forming sound-records from a heated matrix which consists in impacting a comminuted record surfacing material against the matrix, and then associating the surfacing material with a base.
22. The process of forming sound-records from a heated matrix which consists in impacting a heated comminuted record surfacing material against the matrix and then associating the surface with a base.
23. The process of forming sound-records from a matrix which consists in impacting a record surfacing material in comminuted form against a heated matrix to coat the record carrying surface of the matrix with the record surfacing material and subsequently associating the record carrying surfacing material with a base.
24. The process of forming sound-records from a matrix which consists in impacting successive layers of a comminuted record surfacing material against the matrix and on one another and in then associating the
- surfacing material with its sound-record with a base.
25. The process of forming sound-records from a matrix which consists in forcibly 65
- projecting a plastic record surfacing material against the phonetic characters of the matrix to provide the same with a coating, uniting such coating by heat and pressure with a plastic base, subsequent cooling of the 70
- matrix effecting separation of the sound-record from the matrix.
26. The process of forming sound-record tablets from a negative matrix which consists in projecting against the matrix a record surfacing material which has been reduced to fluidity to form a coating on the matrix which coating after solidification and while adhering to the matrix is transferred to a base by pressure and heat.
- 75
27. The process of forming sound-records from a metallic negative which has thereon phonetic characters which consists in projecting a surfacing material containing shell-lac which has been reduced to fluidity by a 80
- solvent against the matrix to coat the same which coating after solidification and while adhering to the matrix is transferred by heat and pressure to a plastic base the record being separated from the matrix by cooling 85
- and a release of pressure.
28. The process of forming sound-records from a metallic negative matrix consisting in projecting a record surfacing material which has been reduced to fluidity with a 90
- force that is sufficient to remove any loose particles on the matrix from the phonetic characters thereof and to provide a coating which while in adherence with the matrix is subjected to heat and pressure to effect 95
- a transfer of the coating to a base.
29. The process of manufacturing sound-records from a matrix which consists as a step in the process in forcibly projecting record surfacing material against the matrix 100
- in a direction that follows the direction of the phonetic characters on the matrix.
30. The process of manufacturing sound-records from a matrix which consists as a step in the process in forcibly projecting 105
- record surfacing material in comminuted form against the matrix, the direction of the projected material being in the general direction of the phonetic characters of the matrix.

EDGAR M. BERLINER.